

Feb. 9, 1937.

W. W. ROWE

2,069,778

PLURAL PLY FABRIC

Filed April 26, 1933



INVENTOR.

William Wallace Rowe

BY

Allen & Allen

ATTORNEY.

## UNITED STATES PATENT OFFICE

2,069,778

## PLURAL PLY FABRIC

William Wallace Rowe, Cincinnati, Ohio, assignor  
to The Paper Service Company, Lockland, Ohio,  
a corporation of Ohio

Application April 26, 1933, Serial No. 668,106

5 Claims. (Cl. 154—50)

My invention relates to plural ply materials comprising creped papers, and more particularly to materials in which the plies comprise a universally stretchable or expansible paper or other web. In the co-pending application of William C. Kemp, Serial No. 558,884, filed August 24, 1931, there is set forth a universally expansible web, characterized by crossing sets of creping crinkles, and while my invention is applicable to any 10 universally stretchable web of paper or the like, yet for many uses I prefer to use the material of the Kemp invention. Another exemplary, but not limiting, instance of a material adapted for use in my invention, is the material set forth in 15 the co-pending application of Rowe and Morris, Ser. No. 622,698, filed July 15, 1932.

My invention relates to structures of or comprising one or more universally stretchable webs joined to similar or dissimilar materials to produce products of novel characteristics. One of 20 the objects of my invention relates to the production of retarded or resisted stretchability in such webs whereby in view of the universally stretchable characteristics thereof, products of unusual physical resistance may be produced. 25 Another object of my invention relates to the production of material in which universally stretchable webs are joined to relatively stiff webs or structures with the production of new effects. Such new effects are of importance in 30 the use of my products as or in connection with wall coverings, floor coverings, container board material etc. Still another object of my invention relates to the production of composite materials and structures comprising at least one 35 stretchable web adhesively joined to a web or structure which is frangible or disintegrable, so as not to localize stretching strains upon the stretchable web.

40 These and other objects of my invention, which will be set forth hereinafter, or will be apparent to one skilled in the art upon reading these specifications, I accomplish by that certain construction and arrangement of parts of which I shall describe certain exemplary embodiments.

Reference is made to the drawing wherein:

Figure 1 is a sectional view of a product comprising a plurality of universally stretchable webs.

50 Fig. 2 is a sectional view of a product comprising a web of universally stretchable material joined to a web of relatively stiff material.

Fig. 3 is a sectional view showing the material of Fig. 2 bent at an angle.

55 Fig. 4 is a perspective view of a product hav-

ing additional means for resisting the removal of stretch.

Fig. 5 is a sectional view of a piece of universally stretchable paper joined to a frangible web.

My invention, likewise, relates to coated webs. 5 The webs may be coated and preferably are coated in the creping process, as may be done in accordance with the teaching of my Re-issue Patent No. 17,633, whereby a product is obtained in which the coating extends well down into the 10 crinkles and in which no separate coating operation is required. My present invention is not, however, limited to webs which are coated prior to or concurrently with a crinkling operation.

One phase of my invention is based upon cer- 15 tain discoveries with respect to the efficacy of coated materials in resisting the stretching of a stretchable web. It is obvious that the force necessary to stretch as well as to tear an uncoated, crinkled web is somewhat less than that 20 necessary to stretch or tear a coated web, since the coating must also be severed or stretched. But I have discovered that coatings upon webs are able to exercise a much more important function in increasing the resistance of a product, as 25 will be shown.

If two pieces of creped paper coated upon one side are simultaneously stretched while not in adhesive juncture, as by placing the two pieces with their paper sides toward each other and 30 their coated sides outwardly disposed, and if the force required to produce a given elongation is measured, a result will be secured which is substantially the sum of the individual resistances of the pieces. If, however, similar coated and 35 creped papers are pressed together with their coated sides in adhesive contact so as to form a composite fabric, then the force required to produce the same elongation will be found to be very greatly increased over the sum of the in- 40 dividual resistances.

While I do not desire to be bound by theory, yet I believe the reason for this phenomenon is as follows: For a clear understanding reference may be made to Fig. 1 wherein I have shown opposed pieces of creped paper indicated at 1 and 2, each of these being coated with, for example, an asphaltic substance in layers indicated at 3 and 4. It may be supposed that the paper has been creped by means of the positive adhesive 45 action of this bitumen, although my product is not so limited. Under these circumstances the bituminous coating will be to all intents and purposes continuous with respect to the paper surface, even within the wrinkles. By reason of the 50

creping action and the forcing of the crinkles together therein the bituminous layer will be thicker in the depressions of the creping than it will be on the peaks thereof. This difference in thickness may be even more pronounced if the asphalt is coated solidly onto previously creped paper. If portions of two such creped webs of material are bonded together as shown, the bond may or may not be continuous, depending upon the amount of coating, and its disposition. There may be interspaces as shown at 5 between the bituminous layers which are fused together elsewhere. In other instances, the crinkles of both sheets may be filled up solid by 15 the coating substance.

Whatever the particular condition of the coating substance between the piles, a stretching of the combined fabric will be manifest not only in an elongation of the webs, and a bending and/or stretching of the coatings thereon, but also in a 20 tendency of the webs to separate, which separation is resisted by the cohesive action of the coating substance. This tendency is primarily due to the non-conjointly creped character of 25 the piles, which produces relative movement of parts as the piles are stretched. In some instances, particularly where the crinkles are filled up more or less solidly with the coating substance, there is a tendency to separate the piles by pulling 30 them apart over relatively incompressible masses of the coating substance. In either event the tendency to separate is strongly resisted by the cohesive force of the coating substance, particularly where the peaks of the crinkles of different piles are joined together by relatively 35 thin films of the coating substance. This action is not found in conjointly creped materials, as where two sheets of plain paper are first cemented together and are then creped as one web, since here the cementitious substance is creped with the paper, and elongates therewith when stretched, and since the paper layers stretch conjointly the cohesive resistance of the cementitious layer is not utilized.

With creped fabrics possessing universal stretchability the phenomenon above discussed is productive of unusual results. In the first place, the fabric has an unusual resistance to the removal of stretch. In the second place, the fabric is unusually serviceable for a number of 40 purposes since a strain placed against the fabric may initially be greater than the ultimate tensile strength of the fabric, but will be compensated for by the controlled elongation thereof. This is set forth in my co-pending application, Serial No. 664,377 filed April 4, 1933, wherein a bag or other flexible container made of such a fabric as I have hereinabove described, is able successfully to withstand stresses which would burst 45 a relatively non-expansile fabric even of very much greater ultimate tensile strength. In the third place, if a relatively continuously plastic coating material is employed, the plies tend to re-cement in new formations and the controlled resistance to the removal of stretch remains at a 50 substantially constant figure throughout a stretching operation which removes less than the total stretchability of the materials. In the fourth place, if the coating substance becomes 55 hard and frangible, it interposes even greater initial resistance to the removal of stretch; and if a stretching action results in a separation of the piles, this does not destroy the utility of the fabric, although its resistance to further stretching may be diminished. The piles will, of course, 60

re-cement if plasticity is restored to the coating. In the fifth place, if a material is employed such as rubber, having a continuous resilience as distinguished from a more or less continuous plasticity, the resistance to the removal of stretch increases as the material is stretched; and when the stretch is relieved the material tends to return to a greater or less degree to its original unstretched condition, as set forth in my co-pending application, Ser. No. 668,105 filed April 10 65 1933. In the sixth place I have found that still greater resistance to the removal of stretch may be obtained by incorporating relatively short and heterogeneously arranged fibers in the coating layer, without destroying the universally stretchable character of that layer. In the seventh place, these products, not only having unusual resistance because of their general stretchability, have unusual properties because of their universal localized stretchability. Thus my 20 fabrics even when made to have relatively great thicknesses can bend back upon themselves sharply without fracture of any of the piles. They are thus of particular utility as floor coverings. That such an action would be impossible 25 in plain felted webs solidly cemented together, is an indication of the utility of my fabrics for use in bending structures alone or in combination with container board or the like which must be scored to be bent. Again the local universal 30 stretchability of my fabrics not only permits them to conform to uneven surfaces, but, as when applied to a wall or the like, enables them to mask a crack and to compensate for subsequent widening or change of shape of the crack. 35

These unusual results are bound up in large measure with the universally stretchable character of the material employed. It may be said that in making materials of this character an initially coated condition of all of the piles is not 40 necessary. A coated ply may be joined to an uncoated ply by means of the coating substance or additional coating substance, and a heightened resistance obtained. However, when using universally stretchable paper the resistance to expansion is greater than when using paper stretchable in but one primary direction, due doubtless to a multi-lateral relative movement of the piles in the stretching operation. Not only this, but a multi-lateral stretchability of the individual 50 webs gives to the product a new usefulness in accommodating itself to uneven surfaces, in the relief of strains by localized as distinguished from general stretchability, in bending around sharp corners, and in embossing. The plural ply 55 fabric of my invention may readily be embossed and will take perfectly very intricate patterns. Likewise, as hereinabove indicated, my material may be bent without cracking and without scoring through a sharp angle by reason of the localized stretchability of the several plies, which under these circumstances move and/or stretch relatively to each other to take up the varying 60 stresses of the bending operation.

Hitherto in the production of articles from boxboard or the like, it has been necessary to score the material where it is to be bent. Such scoring results not only in a separation in the plies but also facilitates the disruption of the outer plies when the board is bent. A composite fabric 70 of a plurality of plies of universally stretchable material made in accordance with my invention may be bent upon itself without scoring and without the disruption of plies. Moreover, one or more plies of coated universally stretchable 75

paper may be joined to relatively stiff materials and the combined structure bent without a disruption of the surface ply at least.

I have shown in Fig. 2 a product comprising the web of universally stretchable paper 7, joined by a coating substance 8 to a web 9 of relatively stiff material such as boxboard or fiber board. When this product is bent as shown in Fig. 3, there is no disruption of the outer ply. The relatively stiff material may be faced on both sides if desired with a coated ply of universally stretchable paper. The universally stretchable paper has in addition the power to accommodate itself to initial surface irregularities of a relatively stiff material or some other support to which it may be applied. Thus panels of stiff material such as board may be covered with a coated layer comprising one or more plies of universally stretchable paper and the ply or plies worked and stretched until it accommodates itself accurately to the surface and to the area to which it is applied. In this way covers may be made for containers of stiff material, applied to the surfaces thereof and worked into continuous surface contact and surface conformation. This function exists not only in single plies but in plural plies of the flexible and universally stretchable material for reasons which have been set forth hereinabove.

30 Likewise completed fabrics comprising plies of universally stretchable material have not only the power to lie flat upon regular surfaces, but also to conform themselves to irregular surfaces. For roofing, siding, wall covering, book binding and the like, my novel product has unusual usefulness.

In Figure 4, I have shown a composite fabric comprising universally stretchable webs 10 and 11, coated with cementing substance as at 12 and 40 13. Relatively short and heterogeneously arranged fibers, as indicated at 14, are placed between the plies so as to be caught by and bonded into the cementing substance. This may be accomplished readily by sprinkling or dusting the fibers upon a coated ply while the coating is in an adhesive condition. An excess of the fibers may be employed, i. e., more than will immediately bond to the coating, and the excess may be removed, immediately, or after further handling of 50 the ply. When a ply has been treated with fibers, another coated ply may be adhesively secured to it, or not, as desired. The addition of fibers, as described, will make a single coating much more resistant to the removal of stretch, and in some instances a firmly adhered coating of heterogeneously arranged fibers upon an external coating will give a desirable surface texture.

The fibers employed may be such as jute, hemp, cotton, or other vegetable or animal fibers, or 60 mineral fibers such as asbestos. By short, I mean varying in length, say from one quarter of an inch or shorter, to two or three inches, although these figures are not limiting. Since they are short and heterogeneously arranged, they retard, but do not 65 destroy the universal stretchability of the coating substance. Upon stress, they will slip with reference to the coating, or will move therein if the coating has a resident plasticity. They increase the resistance of the whole fabric to stretching, 70 without substantially impairing its ultimate stretchability; they increase somewhat the ultimate strength of the fabric; and they make the fabric much more resistant to puncturing.

My invention likewise contemplates the junction of a stretchable web to another web or

material, which whether or not it is itself stretchable, will not act to destroy the stretchability of the stretchable web. Thus in the practice of my invention a stretchable web may be joined to a web which is frangible or disintegrable generally, within the limits of the resistance to stretchability of the combined structure. I have shown in Figure 5, a web of creped paper 15, joined by means of a coating substance 16, to a web 17 of frangible or disintegrable material, such, for example, as a light tissue or a web of loose fibrous material. The tissue, if employed, may have varied characteristics, and may itself be creped or uncreped. It may be so loosely matted or have such inherent stretchability as 15 to yield with the main web, or it may have the property of breaking or disintegrating at a large number of points. In this particular aspect of my invention, however, I distinguish the products last hereinabove described from products in 20 which, for example, a stretchable paper web is joined to a stout plain paper web. In such a product the application of stretching strains will fracture the stout plain paper web at one point or at a small number of points; and upon the 25 continued application of the stretching strain this will result in the preliminary removal of the entire local stretchability of the stretchable web adjacent the fracture, thereby weakening the structure. Some additional stretch may be realized by separation of the plies adjacent the fracture, but this will depend upon the nature of the juncture between webs and the adhesion and cohesion of the cementing agent. A web which, 30 while it may not itself be stretchable, is generally frangible or disintegrable, will not destroy 35 the general stretchability of the combined structure.

A product comprising a web of stretchable material joined by cementing to a web of thin tissue, for example, is useful also as an intermediate stage product in the formation of other structures. Where paper has been creped by means of a bitumen and where it is desired to store it as such, the problem of rendering the coating non-adhesive has been troublesome. The application of a thin tissue to the coated side of such product solves this problem without destroying the general or local stretchability of the paper and without rendering it less suitable for 40 joining to other materials. Where the product is to be joined by additional or a different adhesive to another structure, the fibrous surface formed by the tissue may supply a tooth for the engagement of such adhesive. Where desired, 45 any adhesive used may be caused to strike through the tissue web, which in that instance will act to some extent as a fibrous reinforcement. Where the adhesive does not strike through the frangible web, the web, by splitting, 50 may facilitate separation of plies, which may be desirable in some structures.

It will be understood that modifications can be made in my invention without departing from the spirit thereof.

Having thus described my invention, what I claim as new and desire to secure by Letters Patent, is:—

1. In combination a layer of creped paper of substantial weight and strength, bearing on its 70 surface a layer of adhesive substance, and joined by means of said layer to a thin, tissue-like web, said last mentioned web acting normally to prevent accidental adherence of said adhesive layer to objects, and said last mentioned web be- 75

- ing disintegrable in substantially all its parts when said first mentioned web is stretched so as not to destroy either the local or general stretchability of said layer of creped paper.
5. 2. In combination a layer of creped paper of substantial weight and strength, bearing on its surface a layer of adhesive substance, and joined by means of said layer to a thin, tissue-like web, said last mentioned web acting normally to prevent accidental adherence of said adhesive layer to objects, and said last mentioned web being disintegrable in substantially all its parts when said first mentioned web is stretched so as not to destroy either the local or general stretchability of said layer of creped paper, said layer being permeable to said adhesive when said adhesive is softened to permit the adhesive junction of said combination to a desired substance.
3. In combination, at least one layer of universally stretchable paper of substantial weight and strength adhesively joined to a thin, tissue-like web, said last mentioned web being disintegrable in substantially all its parts when said

first mentioned layer is stretched, so as not to destroy either the local or general stretchability of said layer of universally stretchable paper.

4. In combination, two layers of stretchable paper of substantial weight and strength cemented together by means of an adhesive, and a layer of thin, tissue-like material of fibrous character located therebetween and permeated by said adhesive, said tissue-like material being disintegrable in substantially all its parts when said combination is stretched so as not to destroy either the local or the general stretchability of said layers of stretchable paper.

5. In combination, two layers of stretchable paper of substantial weight and strength cemented together by means of an adhesive, and short, heterogeneously arranged fibrous material located therebetween and substantially permeated by said adhesive, said fibrous material acting to retard but not to destroy either the local or general stretchability of said combination.

WILLIAM WALLACE ROWE.